

# UNITED STATES PATENT OFFICE.

FRANK G. BREYER, OF PALMERTON, PENNSYLVANIA, JAMES A. SINGMASTER, OF BRONXVILLE, NEW YORK, AND ALBERT E. HALL, OF PALMERTON, PENNSYLVANIA, ASSIGNORS TO THE NEW JERSEY ZINC COMPANY, OF NEW YORK, N. Y., A CORPORATION OF NEW JERSEY.

## PRODUCTION OF METAL OXIDS AND OTHER COMPOUNDS OF METALS.

1,322,091.

Specification of Letters Patent. Patented Nov. 18, 1919.

No Drawing.

Application filed August 1, 1919. Serial No. 314,721.

To all whom it may concern:

Be it known that we, FRANK G. BREYER, a citizen of the United States, residing at Palmerton, Carbon county, State of Pennsylvania, JAMES A. SINGMASTER, a citizen of the United States, residing at Bronxville, Westchester county, State of New York, and ALBERT E. HALL, a citizen of the United States, residing at Palmerton, Carbon county, State of Pennsylvania, have invented certain new and useful Improvements in the Production of Metal Oxids and other Compounds of Metals; and we do hereby declare the following to be a full, clear, and exact 15 description of the invention, such as will enable others skilled in the art to which it appertains to make and use the same.

This invention relates to the production of metal oxids or other compounds of metals 20 volatilized by the Wetherill process.

Metallic oxids, such, for example, as zinc 25 oxide and lead zinc oxide, as well as other compounds of metals volatilized by the Wetherill process, such, for example, as basic lead sulfate or sublimed lead, have heretofore been more or less extensively produced by the so-called Wetherill process. In speaking of metals volatilized by the Wetherill process, we intend to describe and 30 cover such metals as are volatilizable at the temperatures attainable in the Wetherill process, and for the sake of brevity, we shall hereinafter designate these metals as volatilizable metals. In the case of certain of such 35 metals, the final or desired compound or compounds thereof are the result of a sequence of actions in which the metalliferous materials of the charge are reduced, the reduced metal volatilized and then oxidized 40 or otherwise compounded, while in other cases a metal compound may be directly volatilized, with or without subsequent oxidation or compounding.

By the expression "Wetherill process" as 45 we have used the same herein, is to be understood the furnacing step of the process for producing metal oxids or other compounds of volatilizable metals in which a charge of the metalliferous material mixed 50 with a reducing agent and spread on an ignited bed of fuel is subjected to a combustion supporting blast or draft and

brought to a sufficiently high temperature to reduce the metalliferous materials and volatilize the reduced metal or metals (and 55 (or) to volatilize a metal or a metal compound or compounds) without bringing the charge to a condition where it becomes impervious to the blast or draft, the entire charge being supported on a furnace hearth 60 or grate designed to hold it without letting any considerable part drop through, and the work-off material being discharged as a clinker or sinter. The "furnacing step" is independent of the subsequent treatment of 65 the laden furnace gases and of the collection of the metal compound or compounds.

As a typical example of the Wetherill process, as heretofore usually practised, we will briefly describe the customary procedure in the commercial production of zinc 70 oxid, including leaded zinc oxid. The furnacing step is generally carried out in a furnace having a broad expanse of horizontal grate or hearth roofed over with an 75 arch, and associated with appropriate instrumentalities for permitting the passage therethrough and into the charge, by either a blast or draft, of a combustion supporting gas. It is customary to first charge upon 80 the furnace grate or hearth a layer of "buckwheat" anthracite coal (which is thereupon ignited, usually by the residual heat of the furnace) and by means of a forced blast or draft of air to bring this initial layer of coal 85 to well-developed combustion. Upon this layer of "bed coal" is then charged the customary mixture or "working charge" characteristic of the Wetherill process, that is to say, a mixture of finely divided reducing coal 90 with the finely divided zinciferous (or zinciferous and plumbiferous) material, such as zinc silicate, roasted zinc blends, roasted so-called "mixed sulfids" of zinc and lead, spelter retort residues, or other reducible zinc-containing or zinc-and-lead containing material at the disposal of the operator. The forced air draft is continued, and, when the familiar flames of greenish tint, known as "zinc candles," begin to make their appearance above the upper surface of the charge, indicating that the reduction and volatilization of the zinc 100 and its oxidation to the form of fume is

well under way, the products of combustion carrying the zinc oxid fume and other volatilized metallic compounds are conveyed through the customary cooling flues, etc., to 5 the bag-room wherein, in a cooled condition, they filter through the bags and pass off into the atmosphere, leaving the fume collected in the interior of the bags, from which it is removed at convenient intervals. The 10 furnace operation is continued until the production of fume therefrom in appreciable quantity ceases, whereupon the residual charge, which is, to a large extent, sintered together, is broken up by long-handled 15 rabbles and pried up and lifted or scraped out through the furnace doors into a receiving pit, or the like, preparatory to the starting of a new operation. The coal or other carbonaceous material of the charge serves 20 the two-fold purpose of furnishing a reducing agent for effecting the reduction of the metalliferous materials of the charge and of furnishing, by combustion, the necessary degree of heat to bring these materials to 25 the reducing temperature characteristic of the process.

As thus ordinarily practised, the above-described furnace operation is attended with certain defects interfering with its full efficiency. Prominent among these defects is the inevitable tendency to the formation of blow-holes or craters at various regions of the charge. These blow-holes represent severally the paths of least resistance for 30 the blast in its passage through the charge and to the extent to which they develop in the progress of the operation they interfere with the uniform distribution of the air in its upward passage and produce "hot spots" 35 representing excessive temperatures as compared with other regions of the charge. From time to time, the workmen endeavor to eliminate these blow holes or hot spots, as far as is feasible, by rabbling the upper 40 surface of the charge, thereby filling in the blow holes or breaking up their continuity; but in spite of the palliative effect of these expedients (which, moreover, consume considerable of the workman's time and attention), it is impossible to obtain uniform 45 working conditions throughout the entire extent of the charge; so that there is not only waste of fuel, and the production locally of higher temperatures than is desirable, but the residues taken from the furnace 50 at the termination of the operation contain notable percentages of zinc. The zinc contained in these residues can not ordinarily be recovered commercially, and, when the 55 residues are employed in the manufacture of spiegeleisen, which may be their destination, the presence of the residual zinc is even objectionable, for the reason that, when volatilized and oxidized in the spiegel- 60 eisen furnace, it interferes to a greater or

less extent with the normal furnace operation and tends to collect in and obstruct the spiegeleisen furnace flues.

A further defect of the above-described furnace practice is that the forced draft, 70 which is employed under relatively considerable pressure, tends to project into the free space above the charge more or less dust, particularly in the region of the blow-holes referred to, and this dusting is further aggravated by the rabbling operations; consequently, in addition to the metallic fume, the products of combustion carry with them from the furnace a notable proportion of dust in the form of fine particles of un-reduced ore, carbon, ash, and the like, which 75 tend to contaminate the fume proper and damage its color and marketability. 80

There are, furthermore, certain requirements of the practice of the Wetherill process 85 as heretofore conducted which hamper the operator in the selection of the quality and size both of the coal and of the zinkiferous material employed in making up the charge. Thus, the requirement that the 90 charge shall be sufficiently permeable for the passage of the air, necessitates the use of a mixture of coal and zinkiferous material of a fairly coarse grade. Serious difficulties are encountered in the use of the smaller 95 sizes of buckwheat coal; and only a fractional part of the zinkiferous constituents of the charge can consist of such extremely finely-divided materials as flotation concentrates, zinc precipitates, flue-dust containing 100 zinc, or the like.

The present invention is designed to improve the practice of the Wetherill process,—particularly in the respects noted. That is to say, to obtain a more uniform distribution of the combustion supporting gas on its way through the charge; to lower the resistance of the charge to the passage of the gas; to avoid the formation of blow holes or hot spots; to minimize the contamination 105 of the fume by dust; to increase the permissible quantity of the working charge and consequently the amount of metalliferous material treated in a given time period; to obtain a more complete extraction of the 110 volatilizable metal values and a saving of fuel per unit of metalliferous material present; to effectively employ cheap coal of extremely small mesh and coal of such low 115 grades as colliery washings, coke breeze, and the like; and to freely utilize metalliferous material of any degree of fineness, including flotation concentrates, finely pulverulent ore, metalliferous precipitates, flue dust, etc. 120

For the attainment of the improved results referred to, we have radically modified the present commercial practice of the Wetherill process. Thus, for the initial step of charging the grate bottom or hearth 125

of the usual oxid furnace with a layer of fine ignition fuel, we have substituted a layer or bed of ignition fuel in the form of briquets. We have found, in actual practice, that it is feasible to employ as the ignition or bed fuel, briquets prepared by compressing finely divided coal, together with a suitable binder (preferably the concentrated waste sulfite liquor of the sulfite paper pulp industry); and that the coal appropriate for the purpose may consist of the cheaper and smaller grades, as, for instance, anthracite coal below the No. 3 buckwheat size,—such as No. 4 buckwheat, colliery washings ("dirt" coal or "dust" coal), coke breeze, etc. We have found that, for this ignition or bed fuel, it is suitable to employ briquets of such size and shape as to materially reduce the resistance to the combustion supporting gas, and nevertheless to supply such a substantially uniform sub-stratum for the support of the superposed working charge as to give free access and practically equal distribution of the gas thereto. Thus, the ignition or bed fuel briquets may be made of a form approximating two pyramids having a common rectangular base of say  $1\frac{1}{2}$  inches on each side, the thickness of the briquets from the apex of one pyramid to the other being say  $1\frac{1}{2}$  inches. In general, the fuel briquets should be of substantially uniform size, and preferably of such shape that they roll or tumble easily over one another. We have found the so-called pillow block, eglette, rounded pillow block, overstuffed pillow, and similar shapes well suited to the purposes of the invention. We have ascertained that when, instead of the usual layer of "buckwheat" anthracite coal, a layer or bed of these fuel briquets is charged upon the grate bottom or hearth of the usual oxid furnace as ignition fuel, the briquets will become ignited by the residual heat of the preceding charge and that they may then be brought to well developed combustion, the working charge may be supplied, without substantially disturbing the original distribution of the ignition briquets, and, consequently, with the preservation of the fairly uniform gas passages which the ignition briquets provide over the entire surface of the hearth for the upward passage of the blast into the working charge. In some instances, such a percentage of metalliferous material may be incorporated in the ignition briquets as may be tolerated without substantially interfering with their normal function, and, to the extent to which this is permissible, the ignition briquets will add a reducing function to their normal ignition function.

A second characteristic feature of the invention consists in making up the working charge of the furnace (that is to say, the reducing agent and the metalliferous mate-

rial) in the form of briquets. This feature of the invention may be practised either by briquetting the metalliferous material alone, without briquetting the reducing agent charged with it; or by briquetting the reducing agent and not briquetting the metalliferous material; or by briquetting the reducing agent and briquetting the metalliferous material separately therefrom; or, preferably by briquetting a mixture of the reducing agent and of the metalliferous material. These briquets may be made of the same shape and dimensions as the fuel briquets hereinbefore referred to, and by the employment of any suitable binder, such as the concentrated waste sulfite liquor described. The reducing agent employed may be of any suitable kind, but one of the marked advantages of the briquetting is that it permits, as we have ascertained, the effective and economical use of reduction coal of the cheaper grades and finer mesh, such as anthracite coal of finer mesh than No. 3 buckwheat, colliery washings, coke breeze, and the like.

A typical procedure, in the manufacture of zinc oxid or leaded zinc oxid, for the production of the working charge briquets made from the preferred mixture of reduction coal and zinkiferous or zinkiferous and plumbiferous material is as follows:

The reduction coal (as, for instance, anthracite "dust" or "slush") which usually averages from 65-70% of carbon (and which usually has a moisture content of about 10%) is placed, together with the sulfite liquor, in a revolving mixer of the kind employed for the mixing of concrete and, after a short period of mixing, the zinkiferous (or zinkiferous and plumbiferous) material is added, and the mixing operation then continued for a further period of three minutes or more. Thus, for 800 pounds of the anthracite dust or slush coal, 67 pounds of concentrated waste sulfite liquor of 30° Baumé is employed, and the metalliferous material added may, for example, consist suitably of 960 pounds of finely crushed zinc ore averaging say 20% of zinc oxid and 16% silica, together with 480 pounds of so-called dust ore averaging say 23% of zinc oxid and 8 to 9% silica,—these ores being, in this instance, mixtures consisting mainly of silicate of zinc, Franklinite and calcite and carrying usually from 1 to 6% of moisture. From the mixer, our practice has been to dump the material directly into a 5 foot dry pan Chilean mill located directly below, and to subject it to the mixing and comminuting action of the mill for three minutes or more. From the Chilean mill, the material is taken to the briquetting press. The "m" of press that we have used to advantage consists of cooperating rolls about 20 inches in diameter and provided with cooperating molding pockets, so that

when the material is fed into the pans of the rolls from above, it is molded into briquets having the shape and dimensions hereinbefore referred to and weighing in the neighborhood of three ounces. The two rolls of the briquetting machine are held together by heavy spring pressure so as to exert a compressive force upon the material as it is being formed into the briquets of about 2,000 pounds to the square inch.

The briquets (averaging between 5% and 10% moisture for the mixed charge and up to say 15% moisture for bed fuel briquets) are placed in baskets which may conveniently be 30 inches long, 20 inches wide and 4 inches high,—the sides of the baskets being of heavy sheet iron and the bottoms of  $\frac{1}{2}$  inch wire mesh. In these baskets, or in similar receptacles, we dry and bake the briquets, as, for instance, by mounting the baskets filled with briquets upon buggies carrying say twelve baskets in four tiers of three baskets each, which are then pushed into a tunnel drier of the direct coal-fired type. The briquets remain in the drier from one to two hours, at a temperature of approximately 200° C. dependent upon the rate of firing. The dried briquets are then removed from the drier, cooled and stored, under cover, for subsequent use. This drying and baking of the briquets is of service to impart to them the desirable amount of resistance to crumbling and breaking, so that they may be freely subjected to the rough handling incident to storing them, conveying them to the furnace, and incident to charging them into the furnace either by hand or otherwise, and so that they may likewise substantially maintain their form during the period that they are giving off their volatilizable metals in the furnace.

While some of the advantages of the invention may be attained by briquetting either the reducing agent or the metalliferous material (or both of them) separately, our preferred practice as above noted, is to make the briquets of a mixture of the reducing agent and the metalliferous material. So also, while the working charge, partly or wholly briquetted, may be used in conjunction with an ignition layer of fine anthracite coal, we prefer to use briquetted ignition fuel in conjunction with a briquetted working charge made up of a briquetted mixture of reducing agent and metalliferous material.

Thus, we have found that when, as in our preferred practice, the working charge, in the form of briquets made up of a mixture of metalliferous material and reducing agent, is charged upon a layer of bed fuel briquets of like shape and dimensions, all of the advantages hereinbefore recited as incident to the invention are present. In other words, the supplying of the working

charge of briquets upon the sub-stratum of well ignited ignition or bed fuel briquets in full combustion builds up within the furnace a total charge of such low resistance to the upward passage of the combustion supporting gas, that the pressure of the blast in the ash pit may be very materially lowered; or, in some cases, it may be supplanted by the suction effect of the ordinary exhaust fan employed in the Wetherill process for withdrawing the fume from the furnace, this exhaust sufficing to pull through the charge a sufficient volume of gas appropriate for the operation.

The process proceeds, without the production of craters or hot spots and with an even distribution of the combustion supporting gas over the entire extent of the charge. It is also found that the reduction and (or) volatilization of zinc, lead, and other volatilizable metallic compounds, as well as the subsequent oxidation and recovery of fume, proceed more completely than in the heretofore customary practice of the Wetherill process, and that the residues show a materially lessened loss of volatilizable metal values.

As a typical instance of the practice of the invention, in the production of zinc oxid, 900 pounds of bed fuel briquets (which may consist entirely of "dust" coal) are spread out as evenly as possible upon an oxid furnace grate of 111 square ft. area. These briquets are then ignited by the residual heat of the furnace from a former operation, and when they have reached a good yellow heat, we charge upon them 8,000 pounds of briquets made from the mixture of reducing coal and zinkiferous material.

A much lighter blow is used, as the process proceeds, than with the heretofore usual Wetherill process charge. The residues are withdrawn in from 6 to 12 hours, the 8 hour period usually giving the best results. The same number of operators is used for withdrawing the residues as for the heretofore ordinary 6,000 pound Wetherill charge, so that for the same labor the charge treated may by the practice of the invention be increased one-third. It is also found that the clinker adheres with very much less tenacity to the furnace walls, so that the exertion required for breaking up the clinker and removing it from the furnace is correspondingly less arduous.

We have hereinbefore referred to the increased capacity of output incident to the invention; and, in this connection, we may state that in the preferred practice of the invention wherein briquets are used for the ignition or bed fuel and briquets of mixed metalliferous material and reducing agent are used, we have been able, with the same expenditure of fuel, to obtain a higher extraction of volatilizable metal values (leav-

ing less volatilizable metals in the residue) than in the heretofore customary Wetherill process practice, and that for a furnace run of the same time-period normally employed 5 in working off the charge of the usual oxid furnace, we have been able as hereinbefore particularly noted, to treat a briqueted charge containing as high as one-third more of metalliferous material than is contained 10 in the heretofore customary Wetherill process working charge.

It will, of course, be understood that the specific examples of typical means of practising the invention are to be understood 15 as illustrative of its practical application, and that they may be widely varied without departing from the intended scope of the invention as more broadly set forth in the general description and in the claims 20 hereunto annexed.

While we have hereinbefore specifically described the invention by reference to the production of zinc oxid, including leaded zinc oxid, we wish it to be understood that 25 the invention is applicable to the production of other metal compounds of the volatilizable metals. In particular, we contemplate the production of basic lead sulfate or sublimed lead by the method of the invention. 30 In general, the procedure for the production of sublimed lead is substantially the same as hereinbefore described, substituting, of course, an appropriate plumbiferous material for the zinciferous material. 35 Thus, for example, the bed fuel or the working charge or both may be briqueted in the manner hereinbefore described and supplied to the furnace hearth in the form of briquets. The working charge consists of a 40 mixture of finely divided galena or native lead sulfid and carbonaceous material or other suitable reducing agent, preferably briqueted as hereinbefore described. The working charge is spread on the ignited 45 layer of bed fuel briquets and upon reaching the reaction temperature, the lead sulfid is reduced and (or) volatilized and subsequently oxidized to lead sulfate and lead oxid, thus forming the so-called basic lead 50 sulfate.

The effluent containing the sublimed lead is withdrawn from the furnace and the metallic product collected in any appropriate manner. As the source of plumbiferous 55 material, we may use a high grade of native lead sulfid suitably crushed and jigged to free it from accompanying gangue material, or we may use lead sulfid concentrates, such as flotation concentrates, or other appropriate 60 plumbiferous-containing material with proper additions of sulfur in the form of pyrite, galena, brimstone or other suitable sulfur-carrying agents, whenever there is a 65 lack of sulfur in the charge to properly sulfate the fume.

What we claim is:—

1. In the production by the Wetherill process of metal oxids or other compounds of volatilizable metals, the step of supplying the bed fuel to the furnace hearth in the 70 form of briquets, substantially as described.

2. In the production by the Wetherill process of metal oxids or other compounds of volatilizable metals, the step of supplying the bed fuel to the furnace hearth in the 75 form of briquets, said briquets containing a percentage of metalliferous material; substantially as described.

3. In the production by the Wetherill process of metal oxids or other compounds 80 of volatilizable metals, the step of supplying in the working charge briqueted metalliferous material; substantially as described.

4. In the production by the Wetherill process of metal oxids or other compounds 85 of volatilizable metals, the step of supplying in the working charge briqueted reducing material; substantially as described.

5. In the production by the Wetherill process of metal oxids or other compounds 90 of volatilizable metals, the step of supplying in the working charge a briqueted mixture of metalliferous material and reducing agent; substantially as described.

6. In the production by the Wetherill process of metal oxids or other compounds 95 of volatilizable metals, the step of supplying the bed fuel in the form of briquets, together with the step of supplying in the working charge briqueted metalliferous material; 100 substantially as described.

7. In the production by the Wetherill process of metal oxids or other compounds 105 of volatilizable metals, the step of supplying the bed fuel in the form of briquets, together with the step of supplying in the working charge briqueted reducing material; substantially as described.

8. In the production by the Wetherill process of metal oxids or other compounds 110 of volatilizable metals, the step of supplying the bed fuel in the form of briquets, together with the step of supplying in the working charge a briqueted mixture of metalliferous material and reducing agent; substantially 115 as described.

9. In the production by the Wetherill process of metal oxids or other compounds of volatilizable metals, the step of supplying the bed fuel in the form of briquets, said 120 briquets containing a percentage of metalliferous material, together with the step of supplying in the working charge briqueted metalliferous material; substantially as described.

10. In the production by the Wetherill process of metal oxids or other compounds of volatilizable metals, the step of supplying the bed fuel in the form of briquets, said 125 briquets containing a percentage of metal- 130

liferous material, together with the step of supplying in the working charge briqueted reducing material; substantially as described.

11. In the production by the Wetherill process of metal oxides or other compounds of volatilizable metals, the step of supplying the bed fuel in the form of briquets, said briquets containing a percentage of metalliferous material, together with the step of supplying in the working charge a briqueted mixture of metalliferous material and reducing agent; substantially as described.

12. In the production of sublimed lead by the Wetherill process, the step of supplying the bed fuel to the furnace hearth in the form of briquets; substantially as described.

13. In the production of sublimed lead by the Wetherill process, the step of supplying the bed fuel to the furnace hearth in the form of briquets, said briquets containing a percentage of plumbiferous material; substantially as described.

14. In the production of sublimed lead by the Wetherill process, the step of supplying in the working charge briqueted plumbiferous material; substantially as described.

15. In the production of sublimed lead by the Wetherill process, the step of supplying in the working charge a briqueted mixture of plumbiferous material and reducing agent; substantially as described.

16. In the production of sublimed lead by the Wetherill process, the step of supplying the bed fuel in the form of briquets, together with the step of supplying in the working charge briqueted plumbiferous material; substantially as described.

17. In the production of sublimed lead by the Wetherill process, the step of supplying the bed fuel in the form of briquets, together with the step of supplying in the working

charge a briqueted mixture of plumbiferous material and reducing agent; substantially as described.

18. In the production of sublimed lead by the Wetherill process, the step of supplying the bed fuel in the form of briquets, said briquets containing a percentage of plumbiferous material, together with the step of supplying in the working charge briqueted plumbiferous material; substantially as described.

19. In the production of sublimed lead by the Wetherill process, the step of supplying the bed fuel in the form of briquets, said briquets containing a percentage of plumbiferous material, together with the step of supplying in the working charge a briqueted mixture of plumbiferous material and reducing agent; substantially as described.

20. In a process for volatilizing and oxidizing metal values involving the blowing of air into a bed containing the metal-bearing material and combustible material under conditions which will leave the worked-off charge as a clinker and which will produce a volatile fume, the step of supplying at least part of the charge in the form of briquets; substantially as described.

21. In the production of sublimed lead involving the blowing of air into a bed containing the metal-bearing material and combustible material under conditions which will leave the worked-off charge as a clinker and which will produce a volatile fume, the step of supplying at least part of the charge in the form of briquets; substantially as described.

In witness whereof we hereunto affix our signatures.

FRANK G. BREYER.  
JAMES A. SINGMASTER.  
ALBERT E. HALL.